



US005409620A

**United States Patent** [19]

Kosal et al.

[11] **Patent Number:** **5,409,620**[45] **Date of Patent:** **Apr. 25, 1995**

[54] **FIBER TREATMENT COMPOSITIONS CONTAINING ORGANOFUNCTIONAL SILOXANES AND METHODS FOR THE PREPARATION THEREOF**

[75] Inventors: **Jeffrey A. Kosal; Diane M Kosal, both of Midland; Anthony Revis, Freeland, all of Mich.**

[73] Assignee: **Dow Corning Corporation, Midland, Mich.**

[21] Appl. No.: **175,807**

[22] Filed: **Dec. 30, 1993**

[51] Int. Cl.<sup>6</sup> ..... **B32B 27/36; D06C 15/00; D06M 11/77**

[52] U.S. Cl. ..... **252/8.6; 252/8.9; 106/287.11; 106/287.12; 106/287.13; 106/287.14; 106/287.15; 106/287.16; 528/15; 528/26; 524/773; 524/765; 524/755; 524/714; 524/792**

[58] **Field of Search** ..... **106/287.11, 287.12, 106/287.13, 287.14, 287.15, 287.16; 252/8.6, 8.9, 308, 315.1, 351, 357, 356; 528/15, 26; 524/773, 765, 755, 714, 792**

[56] **References Cited**

**U.S. PATENT DOCUMENTS**

2,823,218 2/1958 Speier ..... 260/448.2  
3,159,601 12/1964 Ashby ..... 260/46.5  
3,159,602 12/1964 Hamilton ..... 260/61  
3,220,972 11/1965 Lamoreaux ..... 260/46.5  
3,296,291 1/1967 Chalk ..... 260/448.2  
3,419,593 12/1968 Willing ..... 260/448.2  
3,516,946 6/1970 Modic ..... 252/429

3,814,730 6/1974 Karstedt ..... 260/46.5  
3,876,459 4/1975 Burrill ..... 117/141  
3,928,629 12/1975 Chandra ..... 427/387  
4,098,701 7/1978 Burrill ..... 252/8.6  
4,154,714 5/1979 Hockemeyer ..... 260/31.2 R  
4,177,176 12/1979 Burrill ..... 260/29.2  
4,380,367 4/1983 Suzuki ..... 106/287.14  
4,472,551 9/1984 White et al. ..... 524/728  
4,746,750 5/1988 Revis ..... 556/443  
4,933,002 6/1990 Petroff ..... 71/116  
4,954,401 9/1990 Revis ..... 428/412  
4,954,554 9/1990 Bunge ..... 528/338  
4,954,597 9/1990 Revis ..... 528/15  
5,000,861 3/1991 Yang ..... 252/8.6  
5,017,297 5/1991 Spyropoulos ..... 252/8.8  
5,063,260 11/1991 Chen ..... 523/213  
5,066,699 11/1991 Lee ..... 524/379  
5,077,249 12/1991 Lee ..... 502/5  
5,082,735 1/1992 Revis et al. ..... 428/412  
5,095,067 3/1992 Hara et al. ..... 524/506  
5,104,927 4/1992 Hara et al. ..... 524/731  
5,194,460 3/1993 Evans ..... 523/211

*Primary Examiner*—Mark L. Bell

*Assistant Examiner*—C. Bonner

*Attorney, Agent, or Firm*—Timothy J. Troy

[57] **ABSTRACT**

The present invention relates to fiber treatment compositions comprising an unsaturated acetate, an organohydrosiloxane, a metal catalyst, an organosilicon compound, and optionally a dispersant. The compositions of the present invention impart beneficial characteristics such as slickness, softness, compression resistance and water repellency to substrates such as fibers and fabrics.

**28 Claims, No Drawings**

**FIBER TREATMENT COMPOSITIONS  
CONTAINING ORGANOFUNCTIONAL  
SILOXANES AND METHODS FOR THE  
PREPARATION THEREOF**

**BACKGROUND OF THE INVENTION**

The present invention relates to a fiber treatment compositions and to a method of making fiber treatment compositions. More particularly, the present invention relates to organofunctional silicone emulsions and their ability to impart beneficial characteristics such as slickness, softness, compression resistance and water repellency to substrates such as fibers and fabrics that is not possible without the use of the compositions and method of the instant invention.

It is generally known to treat textile fibers with organopolysiloxanes to impart a variety of valuable properties to the fibers, such as water repellency, softness, lubricity, antipilling, good laundry and dry cleaning durability, and the like. The use of organopolysiloxanes to achieve such properties is now well established but there continues to be a need to improve these and other desirable properties of the fibers, especially the antipilling properties of the fabrics made from treated fibers. In particular, there has existed a desire to improve the properties of the fibers while improving the processes by which the organopolysiloxane compositions are applied to the fibers, and in this regard, the need to speed up the processing of the fibers is the most urgently needed.

Typical of prior art compositions and processes used for achieving the desirable processing and end use properties are those curable compositions disclosed in U.S. Pat. No. 3,876,459, issued Apr. 8, 1975 to Burrill in which there is set forth compositions obtained by mixing polydiorganosiloxanes having terminal silicon-bonded hydroxyl radicals with an organosilane (or partial hydrolysates thereof) of the formula  $RSiR'n(X)3-n$ , in which R is a monovalent radical containing at least two amine groups, R' is an alkyl or aryl group, X is an alkoxy radical and n is 0 or 1.

The polydiorganosiloxanes are linear or substantially linear siloxane polymers having terminal silicon-bonded hydroxyl radicals and an average degree of substitution on silicon of 1.9 to 2.0 wherein the substituents are generally methyl radicals. The siloxane polymers have an average molecular weight of at least 750 with the preferred molecular weight being in the range of 20,000 to 90,000. The cure mechanism appears to arise through the reaction of the hydrolyzable groups on the silane with the silanol groups of the siloxane polymer, usually under the influence of a catalyst, and at elevated temperatures.

Burrill discloses in U.S. Pat. No. 4,177,176, issued Dec. 4, 1979, an additional composition for use in treating fibrous materials. The composition is disclosed as containing a polydiorganosiloxane having a molecular weight of at least 2500 and terminal —OX groups in which X is hydrogen, lower alkyl or alkoxyalkyl groups with the proviso that there also be present at least two substituents in the polydiorganosiloxanes which are amine groups. There is also present an organosiloxane having at least three silicon-bonded hydrogen atoms, the curing mechanism being based on the reaction of the silicon-bonded hydrogen atoms with the silanol end

blocks of the polydiorganosiloxane polymers under the influence of a catalyst.

Also included in the prior art is the disclosure of Burrill, et al. in U.S. Pat. No. 4,098,701, issued Jul. 4, 5 1978 in which the inventors set forth yet another curable polysiloxane composition which has been found useful for treating fibers which comprises a polydiorganosiloxane in which at least two siliconbonded substituents contain at least two amino groups, a siloxane 10 having silicon-bonded hydrogen atoms, and a siloxane curing catalyst. A study of the '701 patent shows that "siloxane curing catalyst" is used in the sense that non-siloxane containing organofunctional compounds are used to cure siloxane curable materials, and that siloxane 15 compositions that function as catalysts is not intended.

Also, there is disclosed in the prior art the curable system described by Spyropoulos et al. in European patent application publication 0 358 329 wherein micro-emulsions are described in which the oil phase comprises a reaction product of an organosilicon compound having amino groups and an organosilicon compound having epoxy groups, wherein the reaction product has at least one amino group and two silicon-bonded —OR 20 groups, and a method for making the microemulsions. The organosilicon compound having at least one silicon-bonded substituent of the general formula —R'NHR", wherein R' is a divalent hydrocarbon group having up to 8 carbon atoms, and R" denotes 25 hydrogen, an alkyl group or a group of the general formula —RBH<sub>2</sub>, and (B) an organosilicon compound having at least one substituent of the general formula —R'-Y, wherein R' is as defined for those above, and Y denotes an epoxy group containing moiety, whereby 30 the molar ratio of amino groups in (A) to epoxy groups (B) is greater than 1/1, there being present in the reaction product at least two silicon-bonded —OR groups, wherein R denotes an alkyl, aryl, alkoxyalkyl, alkoxyaryl or aryloxyalkyl groups having up to 8 carbon atoms.

Chen et al., in U.S. Pat. No. 5,063,260 discloses curable silicone compositions which impart beneficial characteristics to fibers, the compositions comprising an amino organofunctional substantially linear polydiorganosiloxane polymer, a blend of an epoxy organofunctional substantially linear polydiorganosiloxane polymer and a carboxylic acid organofunctional substantially linear polydiorganosiloxane polymer, and an aminoorganosilane. Chen et al. also discloses a process for the treatment of animal, cellulosic, and synthetic fibers 45 by applying the composition described above the fiber and thereafter curing the composition on the fiber to obtain a treated fiber.

Yang in European Patent Application No. 0415254 discloses stable aqueous emulsion compositions containing 55 at least two amino functionalized polyorganosiloxane containing one or more silanes and optionally a hydroxy terminated polydiorganosiloxane, textiles treated with the emulsion compositions, and processes for the preparation of the emulsion compositions. Revis in U.S. Pat. Nos. 4,954,401, 4,954,597, and 5,082,735 discloses a coating for a paper substrate produced by contacting 60 and forming a mixture of an allyl ester with at least one methylhydrogensiloxane in the presence of a Group VIII metal catalyst, coating the mixture on the substrate, and heating the mixture of the allyl ester, the methylhydrogensiloxane, the substrate, and the Group VIII metal catalyst in the presence of ambient moisture

until the methylhydrogensiloxane becomes cured and cross-linked.

Bunge in U.S. Pat. No. 4,954,554 discloses aqueous emulsions compositions consisting essentially of a curable silicone composition comprising organopolysiloxane having silicon-bonded hydroxyl radicals or silicon-bonded olefinic radicals, an organohydrogenpolysiloxane and a curing catalyst, a polyvinylalcohol emulsifying agent having a degree of hydrolysis of 90 mole percent or more, and water. These compositions are disclosed as having improved gloss and/or water-repellency and/or adhesive release.

Other silicone emulsions containing olefinic siloxanes have been disclosed. For example, Hara et al. in U.S. Pat. Nos. 5,095,067 and 5,104,927 teaches a release silicone emulsion composition comprising 100 parts by weight of a specific organovinylpolysiloxane, from 1 to 50 parts by weight of a specific organohydrogensiloxane, from 0.5 to 5 parts of a platinum catalyst having a viscosity of 10 centistokes or less at 25° C., from 1.5 to 15 parts by weight of a nonionic emulsifying agent having an average HLB of from 10 to 20, and a pH of 6.5 or less, and water. These compositions are disclosed as having good pot life, curability and that the cured film has good release properties and residual adhesive properties of adhesives.

However, none of the references hereinabove disclose a one component fiber treating emulsion comprising an unsaturated acetate, at least one organohydrogensiloxane, a metal catalyst, an organosilicon compound, and one or more surfactants or solvents which imparts beneficial characteristics to textile fibers.

#### SUMMARY OF THE INVENTION

The instant invention relates to compositions and to improved methods for their use to treat substrates such as fibers and fabrics to enhance the characteristics of the substrates. More specifically, the present invention relates to a fiber treatment composition comprising: (A) an unsaturated acetate; (B) an organohydrogensiloxane; (C) a metal catalyst; and (D) an organosilicon compound.

It has been discovered that a heat activated crosslinking composition consisting of a blend of an unsaturated acetate, an organohydrogensiloxane, a metal catalyst, and an organosilicon compound can be used for the treatments of fibers and fabrics to impart slickness, softness, compression resistance and water repellency to the substrates. The composition remains a fluid until an activation temperature is reached at which point cross-linking occurs.

The present invention further relates to a method of treating a substrate, the method comprising the steps of (I) mixing: (A) an unsaturated acetate, (B) at least one organohydrogensiloxane, (C) a metal catalyst, and (D) an organosilicon compound, and (E) a dispersant selected from the group consisting one or more surfactants and one or more solvents to the mixture of (I), (II) applying the mixture from (I) to a substrate, and (III) heating the substrate.

The present invention also relates to a method of making a fiber treatment composition comprising (I) mixing (i) an organosilicon compound and (ii) a dispersant selected from the group consisting one or more surfactants and one or more solvents, (II) adding to the mixture of (I) a mixture of: (iii) an unsaturated acetate, (iv) at least one organohydrogensiloxane, and (v) a metal catalyst.

It is an object of this invention to provide a fiber treatment composition which imparts slickness, softness, compression resistance, and water repellency to fibers and fabrics.

It is also an object of this invention to provide a fiber treatment composition as a one component stable emulsion composition. It is an additional object of this invention to provide a fiber treatment composition which is non-toxic.

It is an additional object of this invention to provide a fiber treatment composition which has a low cure temperature.

These and other features, objects and advantages of the present invention will be apparent upon consideration of the following detailed description of the invention.

#### DETAILED DESCRIPTION OF THE INVENTION

The present invention relates to a fiber treatment composition comprising: (A) an unsaturated acetate; (B) an organohydrogensiloxane; (C) a metal catalyst; and (D) an organosilicon compound.

Component (A) in the fiber treatment compositions of the instant invention is an unsaturated acetate. The unsaturated acetate can be an allyl ester or vinyl ester such as allyl butyrate, allyl acetate, linallyl acetate, allyl methacrylate, vinyl acetate, allyl acrylate, vinyl butyrate, isopropenyl acetate, vinyl trifluoroacetate, 2-methyl-1-but enyl acetate, vinyl 2-ethyl hexanoate, vinyl 3,5,5-trimethylhexanoate, allyl 3-butenoate, bis-(2-methylallyl)carbonate, diallyl succinate, ethyl diallyl-carbamate, and other known allyl esters. It is preferred for the compositions of the instant invention that the unsaturated acetate is selected from the group consisting of allyl acetate, linallyl acetate, and isopropenyl acetate.

The amount of Component (A) employed in the compositions of the present invention varies depending on the amount of organohydrogensiloxane, metal catalyst, and organosilicon compound that is employed. It is preferred for purposes of this invention that from 0.1 to 50 weight percent of (A), the unsaturated acetate, be used, and it is highly preferred that from 2 to 10 weight percent of unsaturated acetate be employed, said weight percent being based on the total weight of the composition.

Component (B) in the compositions of the present invention is at least one organohydrogensilicon compound which is free of aliphatic unsaturation and contains two or more silicon atoms linked by divalent radicals, an average of from one to two silicon-bonded monovalent radicals per silicon atom and an average of at least one, and preferably two, three or more silicon-bonded hydrogen atoms per molecule thereof. Preferably the organohydrogensiloxane in the compositions of the present invention contains an average of three or more silicon-bonded hydrogen atoms such as, for example, 5, 10, 20, 40, 70, 100, and more.

The organohydrogenpolysiloxane is preferably a compound having the average unit formula  $R_a^1H_bSiO_{(4-a-b)/2}$  wherein  $R^1$  denotes said monovalent radical free of aliphatic unsaturation, the subscript b has a value of from greater than 0 to 1, such as 0.001, 0.01, 0.1 and 1.0, and the sum of the subscripts a plus b has a value of from 1 to 3, such as 1.2, 1.9 and 2.5. Siloxane units in the organohydrogenpolysiloxanes having the average unit formula immediately above have the formulae  $R_3^3SiO_2$ ,

$R_2^3HSiO_3$ ,  $R_2^3SiO_{2/2}$ ,  $R^3HSiO_{2/2}$ ,  $R^3SiO_{3/2}$ ,  $HSiO_{3/2}$  and  $SiO_{4/2}$ . Said siloxane units can be combined in any molecular arrangement such as linear, branched, cyclic and combinations thereof, to provide organohydrogenpolysiloxanes that are useful as component (B) in the compositions of the present invention.

A preferred organohydrogenpolysiloxane for the compositions of this invention is a substantially linear organohydrogenpolysiloxane having the formula  $XR_2SiO(XRSiO)_cSiR_2X$  wherein each R denotes a monovalent hydrocarbon or halohydrocarbon radical free of aliphatic unsaturation and having from 1 to 20 carbon atoms. Monovalent hydrocarbon radicals include alkyl radicals, such as methyl, ethyl, propyl, butyl, hexyl, and octyl; cycloaliphatic radicals, such as cyclohexyl; aryl radicals, such as phenyl, tolyl, and xylyl; aralkyl radicals, such as benzyl and phenylethyl. Highly preferred monovalent hydrocarbon radical for the silicon-containing components of this invention are methyl and phenyl. Monovalent halohydrocarbon radicals free of aliphatic unsaturation include any monovalent hydrocarbon radical noted above which is free of aliphatic unsaturation and has at least one of its hydrogen atoms replaced with a halogen, such as fluorine, chlorine, or bromine. Preferred monovalent halohydrocarbon radicals have the formula  $C_nF_{2n+1}CH_2CH_2$ — wherein the subscript n has a value of from 1 to 10, such as, for example,  $CF_3CH_2CH_2$ — and  $CaF_9CH_2CH_2$ —. The several R radicals can be identical or different, as desired. Additionally, each X denotes a hydrogen atom or an R radical. Of course, at least two X radicals must be hydrogen atoms. The exact value of y depends upon the number and identity of the R radicals; however, for organohydrogenpolysiloxanes containing only methyl radicals as R radicals c will have a value of from about 0 to about 1000.

In terms of preferred monovalent hydrocarbon radicals, examples of organopolysiloxanes of the above formulae which are suitable as the organohydrogenpolysiloxane for the compositions of this invention include  $HMe_2SiO(Me_2SiO)_cSiMe_2H$ ,  $(HMe_2SiO)_4Si$ , cyclo- $MeHSiO$ ,  $(CF_3CH_2CH_2)MeHSiO\{Me(CF_3CH_2CH_2)_cSiO\}_cSiHMe(CH_2CH_2CF_3)$ ,  $Me_3SiO(MeHSiO)_cSiMe_3$ ,  $HMe_2SiO(Me_2SiO)_{0.5c}(MeHSiO)_{0.5c}SiMe_2H$ ,  $HMe_2SiO(Me_2SiO)_{0.5c}(MePhSiO)_{0.1c}(MeHSiO)_{0.4c}SiMe_2H$ ,  $Me_3SiO(Me_2SiO)_{0.3c}(MeHSiO)_{0.7c}SiMe_3$  and  $MeHSi(OSiMe_2H)_3$  organohydrogenpolysiloxanes that are useful as Component (B).

Highly preferred linear organohydrogenpolysiloxanes for the compositions of this invention have the formula  $YMe_2SiO(Me_2SiO)_p(MeYSiO)_qSiMe_2Y$  wherein Y denotes a hydrogen atom or a methyl radical. An average of at least two Y radicals per molecule must be hydrogen atoms. The subscripts p and q can have average values of zero or more and the sum of p plus q has a value equal to c, noted above. The disclosure of U.S. Pat. No. 4,154,714 shows highly-preferred organohydrogenpolysiloxanes.

Especially preferred as Component (B) are methylhydrogensiloxanes selected from the group consisting of bis(trimethylsiloxy)dimethyldihydrogenpolysiloxane, diphenyldimethyldisiloxane, diphenyltetraakis(dimethylsiloxy)disiloxane, heptamethylhydrogenpolysiloxane, hexamethyldihydrogenpolysiloxane, methylhydrogenpolysiloxanes, methyltris(dimethylhydrogenpolysiloxane)silane, pentamethylpentahydrogenpolysiloxane, pentamethylhydrogenpolysiloxane, phenyltris(dimethylhydrogenpolysiloxane)silane, polymethylhydrogenpolysiloxane,

tetrakis(dimethylhydrogenpolysiloxane)silane, tetramethyltetrahydrogenpolysiloxane, tetramethyldihydrogenpolysiloxane, and methylhydrogenpolysiloxane copolymers.

The amount of Component (B) employed in the compositions of the present invention varies depending on the amount of unsaturated acetate, metal catalyst, and organosilicon compound that is employed. It is preferred for purposes of this invention that from 40 to 99.9 weight percent of Component (B) be used, and it is highly preferred that from 70 to 90 weight percent of Component (B) be employed, said weight percent being based on the total weight of the composition.

Component (C) in the compositions of the present invention is a metal catalyst. Preferred metal catalysts for the present invention are the Group VIII metal catalysts and complexes thereof. By Group VIII metal catalyst it is meant herein iron, cobalt, nickel, ruthenium, rhodium, palladium, osmium, iridium and platinum. The metal catalyst of Component (C) can be a platinum containing catalyst component since they are the most widely used and available. Platinum-containing catalysts can be platinum metal, optionally deposited on a carrier, such as silica gel or powdered charcoal; or a compound or complex of a platinum group metal. A preferred platinum-containing catalyst component in the compositions of this invention is a form of chloroplatinic acid, either as the commonly available hexahydrate form or as the anhydrous form, as taught by Speier, U.S. Pat. No. 2,823,218, incorporated herein by reference. A particularly useful form of chloroplatinic acid is that composition obtained when it is reacted with an aliphatically unsaturated organosilicon compound such as divinyldimethyldisiloxane, as disclosed by Willing, U.S. Pat. No. 3,419,593, incorporated herein by reference, because of its easy dispersibility in organosilicon systems. Other platinum catalysts which are useful in the present invention include those disclosed in U.S. Pat. Nos. 3,159,601; 3,159,602; 3,220,972; 3,296,291; 3,516,946; 3,814,730 and 3,928,629, incorporated herein by reference. The preferred Group VIII metal catalyst as Component (C) for the compositions of the present invention is  $RhCl_3$ ,  $RhBr_3$ ,  $RhI_3$ , and complexes thereof, although as described hereinabove other appropriate catalyst systems may be employed such as  $ClRh(PPh_3)_3$  and complexes thereof;  $H_2PtCl_6$ ; a complex of 1,3-divinyl tetramethyl disiloxane and  $H_2PtCl_6$ ; and alkyne complexes of  $H_2PtCl_6$ . A more exhaustive list of appropriate catalyst systems which can be employed as Component (C) in the present invention is set forth in U.S. Pat. No. 4,746,750, which is considered incorporated herein by reference. The Group VII metal catalyst may be complexed with a solvent such as THF (tetrahydrofuran).

Also suitable as a catalyst for Component (C) in the compositions of the instant invention are the novel rhodium catalyst complexes disclosed in copending U.S. application for patent, Ser. No. 08/176,168, filing date Dec. 30, 1993, and assigned to the same assignee as this present application, incorporated herein by reference. These novel rhodium catalyst complexes are generally compositions comprising a rhodium catalyst, an unsaturated acetate such as linallyl acetate, and alcohols having 3 or more carbon atoms including diols, furans having at least one OH group per molecule, and pyrans having at least one OH group per molecule.

The amount of Group VIII metal catalyst, Component (C), that are used in the compositions of this invention

tion is not narrowly limited and can be readily determined by one skilled in the art by routine experimentation. However, the most effective concentration of the Group VIII metal catalyst has been found to be from about one part per million to about two thousand parts per million on a weight basis relative to the unsaturated acetate of Component (A).

Also suitable for use as the metal catalyst Component (C) in the compositions of the instant invention are encapsulated metal catalysts. The encapsulated metal catalyst can be a microencapsulated liquid or solubilized curing catalyst which are prepared by the photoinitiated polymerization of at least one solubilized hydroxyl-containing ethylenically unsaturated organic compound in the presence of a photoinitiator for the polymerization of said compound, an optional surfactant, and a liquid or solubilized curing catalyst for organosiloxane compositions such as the catalysts described by Lee et al. in U.S. Pat. Nos. 5,066,699 and 5,077,249 which are considered incorporated herein by reference. It is preferred for purposes of the present invention that the encapsulated metal catalyst is a microencapsulated curing catalyst prepared by irradiating with UV light in the wavelength range of from 300 to 400 nanometers a solution containing (1) at least one of a specified group of photocrosslinkable organosiloxane compounds derived from propargyl esters of carboxylic acids containing a terminal aromatic hydrocarbon radical and at least two ethylenically unsaturated carbon atoms and (2) a liquid or solubilized hydrosilylation catalyst, such as the catalysts described by Evans et al. in U.S. Pat. No. 5,194,460 and in copending U.S. application for patent, Ser. No. 08/001,607, filing date Jan. 7, 1993, and assigned to the same assignee as this present application, now U.S. Pat. No. 5,279,898, which are considered incorporated herein by reference.

The amount of microencapsulated curing catalyst in the fiber treatment compositions of this invention are typically not restricted as long as there is a sufficient amount to accelerate a curing reaction between components (A) and (B). Because of the small particle size of microencapsulated curing catalysts it is possible to use curing catalyst concentrations equivalent to as little as 1 weight percent or less to as much as 10 weight percent of microencapsulated curing catalyst as Component (C) in the compositions of the present invention, said weight percent being based on the total weight of the composition.

Component (D) in the compositions of this invention is an organosilicon compound having an average of at least one group per molecule selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals having from 2 to 20 carbon atoms, and mixtures thereof. It is preferred for purposes of the present invention that Component (D) is a compound having its formula selected from the group consisting of (i)  $R^{1_3}SiO(R_2SiO)_x(R^1RSiO)_ySiR^{1_3}$ , (ii)  $R_2R^1SiO(R_2SiO)_x(R^1RSiO)_ySiR_2R^1$ , (iii)  $RR^{1_2}SiO(R_2SiO)_x(R^1RSiO)_ySiRR^{1_2}$ , wherein R is a monovalent hydrocarbon or halohydrocarbon radical having from 1 to 20 carbon atoms,  $R^1$  is a group selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radi-

cals having from 2 to 20 carbon atoms, and mixtures thereof, x has a value of 0 to 3000, and y has a value of 1 to 100.

The monovalent radicals of R in Component (D) can contain up to 20 carbon atoms and include halohydrocarbon radicals free of aliphatic unsaturation and hydrocarbon radicals. Monovalent hydrocarbon radicals include alkyl radicals, such as methyl, ethyl, propyl, butyl, hexyl, and octyl; cycloaliphatic radicals, such as cyclohexyl; aryl radicals, such as phenyl, tolyl, and xylyl; aralkyl radicals, such as benzyl and phenylethyl. Highly preferred monovalent hydrocarbon radical for the silicon-containing components of this invention are methyl and phenyl. Monovalent halohydrocarbon radicals include any monovalent hydrocarbon radical noted above which has at least one of its hydrogen atoms replaced with a halogen, such as fluorine, chlorine, or bromine. Preferred monovalent halohydrocarbon radicals have the formula  $C_nF_{2n+1}CH_2CH_2$ — wherein the subscript n has a value of from 1 to 10, such as, for example,  $CF_3CH_2CH_2$ — and  $C_4F_9CH_2CH_2$ —. The several R radicals can be identical or different, as desired and preferably at least 50 percent of all R radicals are methyl.

The functional groups of  $R^1$  are selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals having from 2 to 20 carbon atoms, and mixtures thereof. Hydroxy groups suitable for use in the compositions of the instant invention include hydroxyalkyl groups, hydroxyaryl groups, hydroxycycloalkyl groups, and hydroxycycloaryl groups.

Preferred hydroxy (OH) groups as  $R^1$  in the compositions of this invention include groups such as hydroxy, hydroxypropyl, hydroxybutyl, hydroxyphenyl, hydroxymethylphenyl, hydroxyethylphenyl, and hydroxycyclohexyl.

Carboxy groups suitable for use as  $R^1$  in the compositions of the instant invention include carboxyalkyl groups, carboxyaryl groups, carboxycycloalkyl groups, and carboxycycloaryl groups. Preferred carboxy groups as  $R^1$  in the compositions of this invention include groups such as carboxy, carboxymethyl, carboxyethyl, carboxypropyl, carboxybutyl, carboxyphenyl, carboxymethylphenyl, carboxyethylphenyl, and carboxycyclohexyl.

Ester groups can, also be used as  $R^1$  in the formulae hereinabove. These ester groups can include groups such as alkylesters, arylesters, cycloalkylesters, and cycloarylesters. Preferred ester groups suitable as  $R^1$  in the instant invention are selected from the group consisting of ethyl acetate, methyl acetate, n-propyl acetate, n-butyl acetate, phenyl acetate, benzyl acetate, isobutyl benzoate, ethyl benzoate, ethyl propionate, ethyl stearate, ethyl trimethylacetate, methyl laurate, and ethyl palmitate.

Preferred amino groups as  $R^1$  in the compositions of this invention are exemplified by groups having the formula  $NR_2$  wherein R is hydrogen or a monovalent hydrocarbon radical having from 1 to 20 carbon atoms such as aminoalkyl groups, aminoaryl groups, aminocycloalkyl groups, and aminocycloaryl groups. Preferred amino groups in the instant invention are groups such as amino, aminopropyl, ethylene diaminopropyl, aminophenyl, aminoctadecyl, aminocyclohexyl, propylene diaminopropyl, dimethylamino, and diethylamino.

Acetoxy groups suitable as R<sup>1</sup> in the compositions of the present invention are exemplified by groups having the formula —COOCH<sub>3</sub> such as acetoxyalkyl groups, acetoxyaryl groups, acetoxy(cycloalkyl) groups, and acetoxy(cycloaryl) groups. Preferred acetoxy groups in the compositions of the instant invention include acetoxy, acetoxyethyl, acetoxypropyl, acetoxybutyl, acetoxyphenyl, and acetoxy(cyclohexyl).

Sulfo groups which are preferred as R<sup>1</sup> in the compositions of the present invention are exemplified by groups having the formula SR wherein R is hydrogen or a monovalent hydrocarbon radical having from 1 to 20 carbon atoms such as sulfoalkyl groups, sulfoaryl groups, sulfocycloalkyl groups, and sulfocycloaryl groups. Preferred sulfo groups include hydrogen sulfide, sulfopropyl, methylsulfopropyl, sulfophenyl, and methylsulfo.

Fluoro groups are exemplified by groups such as fluoroalkyl groups, fluoroaryl groups, fluorocycloalkyl groups, and fluorocycloaryl groups. Preferred fluoro groups which are suitable as R<sup>1</sup> in the compositions of this invention include fluoro, fluoropropyl, fluorobutyl, 3,3,3-trifluoropropyl, and 3,3,4,4,5,5,6,6,6-nonafluorohexyl.

Alkoxy groups suitable as R<sup>1</sup> in component (D) of this invention include groups such as alkoxyalkyl groups, alkoxyaryl groups, alkoxy(cycloalkyl) groups, and alkoxy(cycloaryl) groups. Preferred alkoxy groups for R<sup>1</sup> in the present invention are groups such as methoxy, ethoxy, butoxy, tertiary-butoxy, propoxy, isopropoxy, methoxyphenyl, ethoxyphenyl, methoxybutyl, and methoxypropyl groups.

Epoxy groups suitable as R<sup>1</sup> in component (D) of this invention include groups such as epoxyalkyl groups, epoxyaryl groups, epoxycycloalkyl groups, and epoxycycloaryl groups. Preferred epoxy groups for R<sup>1</sup> in the present invention are groups such as epoxide, epichlorohydrin, ethylene oxide, epoxybutane, epoxycyclohexane, epoxyethylhexanol, epoxy propanol, and epoxy resin groups.

Acrylate groups suitable as R<sup>1</sup> in the formulae hereinabove include groups such as acryloxy, acryloxyalkyl groups, acryloxyaryl groups, acryloxy(cycloalkyl) groups, and acryloxy(cycloaryl) groups. Preferred acrylate groups suitable as R<sup>1</sup> in the instant invention are selected from the group consisting of acryloxyethyl, acryloxyethoxy, acryloxypropyl, acryloxypropoxy, methacryloxyethyl, methacryloxyethoxy, methacryloxypropyl, and methacryloxypropoxy.

Ether groups can also be used as R<sup>1</sup> in the formulae hereinabove. These ether groups can include groups such as alkylethers, arylethers, cycloalkylethers, and cycloarylethers. Preferred ether groups suitable as R<sup>1</sup> in the instant invention are selected from the group consisting of methylethylether, methylpropylether, ethylmethylether, ethylethylether, ethylpropylether, methylphenylether, ethylphenylether, isopropylphenylether, tertiary-butylpropylether, methylcyclohexylether, and ethylcyclohexylether.

The olefinic hydrocarbon radicals of R<sup>1</sup> of the present invention may have from 2 to 20 carbon atoms. The olefinic hydrocarbon radicals are preferably selected from the group consisting of the vinyl radical and higher alkenyl radicals represented by the formula —R(CH<sub>2</sub>)<sub>m</sub>CH=CH<sub>2</sub> wherein R denotes —(CH<sub>2</sub>)<sub>n</sub>— or —(CH<sub>2</sub>)<sub>p</sub>CH=CH— and m has the value of 1, 2, or 3, n has the value of 3 or 6, and p has the value of 3, 4, or 5. The higher alkenyl radicals represented by the

formula —R(CH<sub>2</sub>)<sub>m</sub>CH=CH<sub>2</sub> contain at least 6 carbon atoms. For example, when R denotes —(CH<sub>2</sub>)<sub>n</sub>—, the higher alkenyl radicals include 5-hexenyl, 6-heptenyl, 7-octenyl, 8-nonenyl, 9-decenyl, and 10-undecenyl. When R denotes —(CH<sub>2</sub>)<sub>p</sub>CH=CH—, the higher alkenyl radicals include, among others, 4,7-octadienyl, 5,8-nonadienyl, 5,9-decadienyl, 6,11-dodecadienyl and 4,8-nonadienyl. Alkenyl radicals selected from the group consisting of 5-hexenyl, 7-octenyl, 9-decenyl, and 5,9-decadienyl, are preferred. It is more preferred that R denote —(CH<sub>2</sub>)<sub>n</sub>— so that the radicals contain only terminal unsaturation and the most preferred radicals are the vinyl radical and the 5-hexenyl radical.

Specific examples of preferred polydiorganosiloxanes

15 for use as Component (D) in the compositions of the present invention include ViMe<sub>2</sub>SiO(Me<sub>2</sub>SiO)<sub>x</sub>SiMe<sub>2</sub>Vi, HexMe<sub>2</sub>SiO(Me<sub>2</sub>SiO)<sub>x</sub>(MeHexSiO)<sub>y</sub>SiMe<sub>2</sub>Hex, ViMe<sub>2</sub>SiO(Me<sub>2</sub>SiO)<sub>x</sub>(MeViSiO)<sub>y</sub>SiMe<sub>2</sub>Vi, HexMe<sub>2</sub>SiO(Me<sub>2</sub>SiO)<sub>196</sub>(MeHexSiO)<sub>4</sub>SiMe<sub>2</sub>Hex, HexMe<sub>2</sub>SiO(Me<sub>2</sub>SiO)<sub>198</sub>(MeHexSiO)<sub>2</sub>SiMe<sub>2</sub>Hex, HexMe<sub>2</sub>SiO(Me<sub>2</sub>SiO)<sub>151</sub>(MeHexSiO)<sub>3</sub>SiMe<sub>2</sub>Hex, and ViMe<sub>2</sub>SiO(Me<sub>2</sub>SiO)<sub>96</sub>(MeViSiO)<sub>2</sub>SiMe<sub>2</sub>Vi, HexMe<sub>2</sub>SiO(Me<sub>2</sub>SiO)<sub>x</sub>SiMe<sub>2</sub>Hex, PhMeViSiO(Me<sub>2</sub>SiO)<sub>x</sub>SiPhMeVi, HexMe<sub>2</sub>SiO(Me<sub>2</sub>SiO)<sub>130</sub>SiMe<sub>2</sub>Hex, ViMePhSiO(Me<sub>2</sub>SiO)<sub>145</sub>SiPhMeVi, ViMe<sub>2</sub>SiO(Me<sub>2</sub>SiO)<sub>299</sub>SiMe<sub>2</sub>Vi, ViMe<sub>2</sub>SiO(Me<sub>2</sub>SiO)<sub>800</sub>SiMe<sub>2</sub>Vi, ViMe<sub>2</sub>SiO(Me<sub>2</sub>SiO)<sub>30</sub>SiMe<sub>2</sub>Vi, ViMe<sub>2</sub>SiO(Me<sub>2</sub>SiO)<sub>198</sub>SiMe<sub>2</sub>Vi, vinyldimethylsiloxy-terminated poly((3,3,3-trifluoropropyl)methylsiloxy)pentasiloxane, vinylmethylsiloxy-terminated polydimethylsiloxane having (3,3,4,4,5,5,6,6,6-nonafluorobutyl)methylsiloxy functional groups. vinyldimethylsiloxy-terminated polydimethylsiloxane having (3,3,3-trifluoropropyl)methylsiloxy groups, vinylmethylsiloxy-terminated polydimethylsiloxane having (3,3,4,4,5,5,6,6,6-nonafluorobutyl)methylsiloxy functional groups, dimethylhydridosiloxy-terminated poly((3,3,3-trifluoropropyl)methylsiloxy)pentasiloxane, dimethylhydroxysiloxy-terminated polydimethylsiloxane, and dimethylhydroxysiloxy-terminated dimethyl(aminoethylaminopropyl)methyl siloxane, wherein Me, Vi, Hex, and Ph denote methyl, vinyl, 5-hexenyl and phenyl, respectively.

45 The amount of Component (D) employed in the compositions of the present invention varies depending on the amount of organohydrogensiloxane, metal catalyst, and unsaturated acetate, that is employed. It is preferred for purposes of this invention that from 1 to 99 weight percent of (D), the organosilicon compound, be used, and it is highly preferred that from 70 to 95 weight percent of (D) be employed, said weight percent being based on the total weight of the composition.

50 The compositions of the instant invention can further comprise (E) a dispersant selected from the group consisting of one or more surfactants and one or more solvents. The (emulsifying agents) surfactants are preferably of the non-ionic or cationic types and may be employed separately or in combinations of two or more. Suitable emulsifying agents for the preparation of a stable aqueous emulsion are known in the art. Examples of nonionic surfactants suitable as component (E) of the present invention include polyoxyethylene alkyl ethers, polyoxyethylene alkylphenol ethers, polyoxyethylene lauryl ethers and polyoxyethylene sorbitan monolaurates such as Brij TM 35L (from ICI Americas Inc., Wilmington, Del. 19897), Brij TM 30 (ICI Americas Inc., Wilmington, Del. 19897), and Tween TM 80 (ICI Americas Inc., Wilmington, Del. 19897), polyoxyethylene alkyl esters, polyoxyethylene sorbitan alkyl esters, polyethyl-

ene glycol, polypropylene glycol, ethoxylated trimethylnonyanois such as Tergitol® TMN-6 (from Union Carbide Chem. & Plastics Co., Industrial Chemicals Div., Danbury, Conn. 06817-0001), and polyoxyalkylene glycol modified polysiloxane surfactants. Examples of cationic surfactants suitable as component (E) in the compositions of the instant invention include quaternary ammonium salts such as alkyltrimethylammonium hydroxide, dialkyldimethylammonium hydroxide, methylpolyoxyethylene cocoammonium chloride, and diplmityl hydroxyethylammonium methosulfate. Preferably, a combination of two or three nonionic surfactants, or a combination of a cationic surfactant and one or two nonionic surfactants are used to prepare the emulsions of the present invention.

Examples of the preferred surfactants for use as Component (E) in the compositions of this invention are the reaction products of alcohols and phenols with ethylene oxide such as the polyethoxyethers of nonyl phenol and octyl phenol and the trimethylol ethers of polyethylene glycols, monoesters of alcohols and fatty acids such as glycerol monostearate and sorbitan monolaurate, and the ethoxylated amines such as those represented by the general formula



in which  $\text{R}'''$  is an alkyl group having from about 12 to about 18 carbon atoms and the sum of  $a$  and  $b$  is from 2 to about 15. Silicone surfactants are also suitable for use as Component (E) in the instant invention. Preferred silicone surfactants include silicone polyethers such as polyalkylpolyether siloxanes and silicone glycol surfactants including silicone glycol polymers and copolymers such as those disclosed in U.S. Pat. No. 4,933,002, incorporated herein by reference. The emulsifying agents may be employed in proportions conventional for the emulsification of siloxanes, from about 1 to about 30 weight percent, based on the total weight of the composition.

Solvents may also be employed as Component (E) in the compositions of the instant invention. Preferred solvents for use as Component (E) in the instant invention include hydrocarbon solvents such as dichloromethane (methylene chloride) and acetonitrile. It is preferred for purposes of the present invention that Component (E), the dispersant, be a mixture of water and one or more of the surfactants described hereinabove. It is also preferred that emulsification of the compositions of the instant invention is carried out by adding one or more emulsifying agents, and water be added to components (A), (B), (C), and (D) described hereinabove and the resulting composition be subjected to high shear.

The amount of Component (E) employed in the compositions of the present invention varies depending on the amount of organohydrogensiloxane, metal catalyst, unsaturated acetate, and organosilicon compound that is employed. It is preferred for purposes of this invention that from 0.25 to 99 weight percent of (E), the dispersant, be used, and it is highly preferred that from 1 to 95 weight percent of dispersant be employed, said weight percent being based on the total weight of the composition. When a surfactant is employed it is preferred that from 0.25 to 20 weight percent be used, and

when a solvent is employed it is preferred that from 70 to 99.5 weight percent be used, said weight percent being based on the total weight of the composition.

The present invention further relates to a method of treating a substrate, the method comprising the steps of (I) mixing: (A) an unsaturated acetate, (B) at least one organohydrogensiloxane, (C) a metal catalyst, (D) an organosilicon compound having an average of at least one group per molecule selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals having from 2 to 20 carbon atoms, and mixtures thereof, and (E) a dispersant selected from the group consisting of one or more surfactants and one or more solvents, (II) applying the mixture from (I) to a substrate, and (III) heating the substrate. Components (A), (B), (C), (D), and (E) are as delineated above including preferred amounts and embodiments thereof.

The present invention also relates to a method of making a fiber treatment composition comprising (I) mixing (A) an unsaturated acetate, (B) at least one organohydrogensiloxane, (C) a metal catalyst, (D) an organosilicon compound having an average of at least one group per molecule selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals having from 2 to 20 carbon atoms, and mixtures thereof, and (E) a dispersant selected from the group consisting of one or more surfactants and one or more solvents. Again, Components (A), (B), (C), (D), and (E) are as delineated above including preferred amounts and embodiments thereof.

The present invention further relates to a method of making a fiber treatment composition comprising: (I) mixing: (i) an organosilicon compound having an average of at least one group per molecule selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals having from 2 to 20 carbon atoms, and mixtures thereof, and (ii) a dispersant selected from the group consisting of one or more surfactants and one or more solvents; (II) adding to the mixture of (I) a mixture of: (iii) an unsaturated acetate, (iv) at least one organohydrogensiloxane, and (v) a metal catalyst. The mixture of Step (II) can be emulsified prior to adding the mixture of (II) to the mixture of (I). Again, Components (A), (B), (C), (D), and the surfactants are as delineated above including preferred amounts and embodiments thereof.

The compositions comprising components (A), (B), (C), (D), and optionally any surfactants or solvents (E) may be applied to the fibers by employing any suitable application technique, for example by padding or spraying, or from a bath. For purposes of this invention, the compositions can be applied from a solvent, but is preferred that the compositions be applied from an aqueous medium, for example, an aqueous emulsion. Thus, any organic solvent can be employed to prepare the solvent-based compositions, it being understood that those solvents that are easily volatilized at temperatures of from room temperatures to less than 100°C. are preferred,

for example, such solvents may include methylene chloride, acetonitrile, toluene, xylene, white spirits, chlorinated hydrocarbons, and the like. The treating solutions can be prepared by merely mixing the components together with the solvent. The concentration of the treating solution will depend on the desired level of application of siloxane to the fiber, and on the method of application employed, but it is believed by the inventors herein that the most effective amount of the composition should be in the range such that the fiber (or fabric) picks up the silicone composition at about 0.05% to 10% on the weight of the fiber or fabric. According to the instant inventive method of treatment, the fibers usually in the form of tow, or knitted or woven fabrics, are immersed in an aqueous emulsion of the compositions whereby the composition becomes selectively deposited on the fibers. The deposition of the composition on the fibers may also be expedited by increasing the temperatures of the aqueous emulsion, temperatures in the range of from 20° to 60° C. being generally preferred.

Preparation of the aqueous emulsions can be carried out by any conventional technique. The compositions of this can be prepared by homogeneously mixing Components (A), (B), (C), and (D) and any optional components in any order. Thus it is possible to mix all components in one mixing step immediately prior to using the fiber treatment compositions of the present invention. Most preferably (A), (B), and (C) are emulsified and then (D) is emulsified and the two emulsions thereafter combined. The emulsions of the present invention may be macroemulsions or microemulsions and may also contain optional ingredients, for example antifreeze additives, preservatives, biocides, organic softeners, antistatic agents, dyes and flame retardants. Preferred preservatives include Kathon ® LX (5-chloro-2-methyl-4-isothiazolin-3-one from Rohm and Haas, Philadelphia, Pa. 19106), Giv-gard ® DXN (6-acetoxy-2,4-dimethyl-m-dioxane from Givaudan Corp., Clifton N.J. 07014), Tektamer ® A.D. (from Calgon Corp., Pittsburgh, Pa. 152300), Nuosept ® 91.95 (from Huls America, Inc., Piscataway, N.J. 08854), Germaben ® (diazolidinyl urea and parabens from Sutton Laboratories, Chatham, N.J. 07928), Proxel ® (from ICI Americas Inc., Wilmington, Del. 19897), methyl paraben, propyl paraben, sorbic acid, benzoic acid, and lauricidin.

Following the application of the siloxane composition to the substrate, the siloxane is then cured. Preferably, curing is expedited by exposing the treated fibers to elevated temperatures, preferably from 50° to 200° C.

The compositions of this invention can be employed for the treatment of substrates such as animal fibers such as wool, cellulosic fibers such as cotton, and synthetic fibers such as nylon, polyester and acrylic fibers, or blends of these materials, for example, polyester/cotton blends, and may also be used in the treatment of leather, paper, and gypsum board. The fibers may be treated in any form, for example as knitted and woven fabrics and as piece goods. They may also be treated as agglomerations of random fibers as in filling materials for pillows and the like such as fiberfil.

The composition of components (A), (B), (C), and (D) should be used at about 0.05 to 25 weight percent in the final bath for exhaust method applications, and about 5 gm/l to 80 gm/l in a padding method of application, and about 5 gm/l to 600 gm/l for a spraying application. The compositions employed in this process are

particularly suitable for application to the fibers or fabrics from an aqueous carrier. The compositions can be made highly substantive to the fibers, that is they can be made to deposit selectively on such fibers when applied thereto as aqueous emulsions. Such a property renders the compositions particularly suited for aqueous batch treatment by an exhaustion procedure, such exhaustion procedures being known to those skilled in the art. The compositions of the instant invention are new and novel and provide a fast cure and wide cure temperature ranges for curing them on fibers or fabrics compared to the compositions of the prior art, having a temperature cure range of from 50° C. to 200° C. Further, the fibers have superior slickness and no oily feeling after cure. The compositions of the instant invention provide consistent performance, good bath life of more than 24 hours at 40° C., have good laundry and dry cleaning durability, and have very good suitability for application by spraying.

Fiber Slickness was tested by using a DuPont ® unslickened fiberfil product, i.e. Hollofil ® T-808, for the evaluation of slickness imparted by the application of the silicone emulsion of the present invention. A piece of Hollofil ® T-808 is soaked in the diluted emulsion of interest and then passed through a roller to obtain 100% wet-pickup, i.e., the weight of the finished fiberfil is twice that of the unfinished fiberfil. After drying at room temperature, the finished sample is heated at 175° C. for 2-25 minutes. Thus prepared, the finished fiberfil usually contains approximately the same silicone level as that of the emulsion of interest.

The slickness of fiberfil is measured by staple pad friction which is determined from the force required to pull a certain weight over a fiberfil staple pad. The staple pad friction is defined as the ratio of the force over the applied weight. A 10 pound weight was used in the friction measurement of this invention. A typical instrument set-up includes a friction table which is mounted on the crosshead of an Instron tensile tester. The friction table and the base of the weight are covered with Emery Paper #320 from the 3M Company so that there is little relative movement between the staple pad and the weight or the table. Essentially all of the movement is a result of fibers sliding across each other. The weight is attached to a stainless steel wire which runs through a pulley mounted at the base of the Instron tester. The other end of the stainless steel wire is tied to the loadcell of the Instron tester.

Following are examples illustrating the compositions and methods of the present invention. In the examples hereinbelow, THF denotes tetrahydrofuran, THFA denotes tetrahydrofurfuryl alcohol, and TPRh denotes  $(Ph_3P)_3RhCl_3$  (tris-(triphenylphosphine)rhodium chloride).

In the examples hereinbelow, a variety of different organosilicon compounds were used in preparing the compositions of the instant invention. Each organosilicon compound is delineated below and is designated by a corresponding letter. The letters then appear in Tables I and II below thus designating the type of organosilicon compound employed.

A—a 9,500 cps vinyldimethylsiloxy-terminated polydimethylsiloxane.

B—a 40,000 cps polydimethylsiloxane having 30% pendant vinylmethylsiloxy moieties.

C1—Silicone in water emulsion of 65 micron diameter particle size containing vinyldimethylsiloxy-ter-

minated poly((3,3,3-trifluoropropyl)methylsiloxy)pentasiloxane.

C2—Silicone in water emulsion of 2 micron diameter particle size containing vinyldimethylsiloxy-terminated poly((3,3,3-trifluoropropyl)methylsiloxy)pentasiloxane.

D—Silicone in water emulsion containing 30,000 cps vinylmethylsiloxy-terminated polydimethylsiloxy having 30% (3,3,4,4,5,5,6,6,6-nonafluorobutyl)methylsiloxy moieties.

E—Silicone in water emulsion containing vinyldimethylsiloxy-terminated polydimethylsiloxydodecasiloxane having 40% (3,3,3-trifluoropropyl)methylsiloxy moieties.

F—Silicone in water emulsion containing 10,000 cps vinylmethylsiloxy-terminated polydimethylsiloxy having 30% (3,3,4,4,5,5,6,6,6-nonafluorobutyl)methylsiloxy moieties.

G—Silicone in water emulsion containing dimethylhydridosiloxy-terminated poly((3,3,3-trifluoropropyl)methylsiloxy)pentasiloxane.

H—Silicone in water emulsion containing 1,500,000 cps dimethylhydroxysiloxy-terminated polydimethylsiloxy.

I—Silicone in water emulsion containing 12,500 cps dimethylhydroxysiloxy-terminated polydimethylsiloxy.

5 compound (denoted in Table I hereinbelow) was added to the mixture and stirred gently until the mixture was again homogenous. This was followed by adding about 1.78 grams of a polyoxyethylene lauryl ether surfactant or a methylene chloride solvent (in Example 7 a solvent was substituted for the surfactant), and about 38 grams of water containing up to about 0.22 grams of a preservative (sorbic acid) to the mixture. Mixing was then resumed at medium speed for 20 to 30 minutes. The mixture was then processed through a high shear device to produce the emulsions of the instant invention. The particle sizes of the emulsions ranged from 0.7 to 3.0 microns and the pH of the emulsions ranged from 3.0 to 4.5.

10 15 A relative ranking from 1 to 10 was established using known commercial finishes based upon slickness values obtained using the Staple Pad Friction frictional test described hereinabove. No finish was given a ranking of 1, the commercial finish was given a ranking of 6, and a premium finish was given a ranking of 10. The amount of organosilicon compound, organosilicon compound type, the amount of linallyl acetate, the amount of catalyst, catalyst type, the time it took each sample to cure in minutes (min.), and the performance of each example 20 25 are reported in Table I hereinbelow.

TABLE I

| Organosilicon Compound |    | Example | Type | Amount (g) | Linallyl Acetate (g) | Catalyst (g)             | Catalyst Type | Cure (Min.) | Rating |
|------------------------|----|---------|------|------------|----------------------|--------------------------|---------------|-------------|--------|
|                        |    |         |      |            |                      |                          |               |             |        |
| 1                      | A  | 10      |      | 10         | 0.1                  | RhCl <sub>3</sub> , THF  | 5             | 10          |        |
| 2                      | C1 | 3       |      | 3          | 0.1                  | RhCl <sub>3</sub> , THF  | 10            | 10          |        |
| 3                      | C2 | 3       |      | 3          | 0.1                  | RhCl <sub>3</sub> , THF  | 10            | 8           |        |
| 4                      | A  | 10      |      | 10         | 0.3                  | 10% Pt, Linallyl         | 8             | 11          |        |
| 5                      | B  | 10      |      | 0          | 0.3                  | 1% Pt, Linallyl          | 3             | 11          |        |
| 6                      | D  | 2.5     |      | 0          | 0.3                  | 1% Pt, Linallyl          | 15            | 9           |        |
| 7                      | E  | 3       |      | 0          | 0.3                  | 1% Pt, Linallyl          | 10            | 9           |        |
| 8                      | F  | 3       |      | 0          | 0.3                  | 1% Pt, Linallyl          | 10            | 11          |        |
| 9                      | G  | 2       |      | 0          | 0.3                  | 1% Pt, Linallyl          | 14            | 11          |        |
| 10                     | K  | 10      |      | 4          | 0.1                  | RhCl <sub>3</sub> , THFA | 10            | 10          |        |

J—Silicone in water emulsion containing 4,000 cps dimethylhydroxysiloxy-terminated dimethyl(aminooethylaminopropyl)methyl siloxane.

K—a 250 cps polydimethylsiloxy having 8% pendant alkylsulfocarboxy moieties.

45 The examples in Table I hereinabove show that the organosilicon compounds of the instant invention cure into fiber treatment compositions to give good slickness ratings.

## EXAMPLES 11-13

Another fiber treatment composition was prepared by preparing a first solution by mixing 33 grams of a trimethylsilyl terminated polymethylhydrogensiloxane 50 having a viscosity of 30 centistokes at a temperature of 25° C. and having the formula Me<sub>3</sub>SiO(MeHSiO)<sub>7</sub>OSiMe<sub>3</sub>, 2 grams of linallyl acetate, and 0.03 grams of TPRh with 60 grams of water containing 4.8 grams of a nonionic polyoxyethylene lauryl ether surfactant and stirring. This mixture was then subjected to high shear until the desired emulsion particle size was attained.

A second solution was prepared by mixing 35 grams of an organosilicon compound (denoted in Table II) with 60 grams of water containing 4.8 grams of a non-ionic polyoxyethylene lauryl ether surfactant and about 0.3 grams of a preservative (sorbic acid) and stirring. This mixture was then subjected to high shear until the desired emulsion particle size was attained.

60 65 In examples 11 and 12, 10 parts of the first solution was mixed with 90 parts of the second solution and the resulting mixture was stirred. In example 13, 3 parts of the first solution was mixed with 97 parts of the second solution and the resulting mixture was stirred. The typi-

EXAMPLES 1-10

In order to illustrate the effectiveness of the compositions of the present invention the following tests were conducted. Two catalysts were prepared, a rhodium catalyst and a microencapsulated curing catalyst. A .03 molar rhodium catalyst solution was prepared by dissolving 1 gram of RhCl<sub>3</sub>·6H<sub>2</sub>O (rhodium trichloride hexahydrate) or TPRh in 120 grams of THF, THFA, or linallyl acetate. A 10% and 1% platinum catalyst solution was prepared by dissolving 10 grams and 1 gram, respectively, of a platinum catalyst prepared according to Example 3 of U.S. Pat. No. 5,194,460 in 90 grams and 99 grams, respectively, of linallyl acetate.

65 70 75 80 85 90 95 100 105 110 115 120 125 130 135 140 145 150 155 160 165 170 175 180 185 190 195 200 205 210 215 220 225 230 235 240 245 250 255 260 265 270 275 280 285 290 295 300 305 310 315 320 325 330 335 340 345 350 355 360 365 370 375 380 385 390 395 400 405 410 415 420 425 430 435 440 445 450 455 460 465 470 475 480 485 490 495 500 505 510 515 520 525 530 535 540 545 550 555 560 565 570 575 580 585 590 595 600 605 610 615 620 625 630 635 640 645 650 655 660 665 670 675 680 685 690 695 700 705 710 715 720 725 730 735 740 745 750 755 760 765 770 775 780 785 790 795 800 805 810 815 820 825 830 835 840 845 850 855 860 865 870 875 880 885 890 895 900 905 910 915 920 925 930 935 940 945 950 955 960 965 970 975 980 985 990 995 1000 1005 1010 1015 1020 1025 1030 1035 1040 1045 1050 1055 1060 1065 1070 1075 1080 1085 1090 1095 1100 1105 1110 1115 1120 1125 1130 1135 1140 1145 1150 1155 1160 1165 1170 1175 1180 1185 1190 1195 1200 1205 1210 1215 1220 1225 1230 1235 1240 1245 1250 1255 1260 1265 1270 1275 1280 1285 1290 1295 1300 1305 1310 1315 1320 1325 1330 1335 1340 1345 1350 1355 1360 1365 1370 1375 1380 1385 1390 1395 1400 1405 1410 1415 1420 1425 1430 1435 1440 1445 1450 1455 1460 1465 1470 1475 1480 1485 1490 1495 1500 1505 1510 1515 1520 1525 1530 1535 1540 1545 1550 1555 1560 1565 1570 1575 1580 1585 1590 1595 1600 1605 1610 1615 1620 1625 1630 1635 1640 1645 1650 1655 1660 1665 1670 1675 1680 1685 1690 1695 1700 1705 1710 1715 1720 1725 1730 1735 1740 1745 1750 1755 1760 1765 1770 1775 1780 1785 1790 1795 1800 1805 1810 1815 1820 1825 1830 1835 1840 1845 1850 1855 1860 1865 1870 1875 1880 1885 1890 1895 1900 1905 1910 1915 1920 1925 1930 1935 1940 1945 1950 1955 1960 1965 1970 1975 1980 1985 1990 1995 2000 2005 2010 2015 2020 2025 2030 2035 2040 2045 2050 2055 2060 2065 2070 2075 2080 2085 2090 2095 2100 2105 2110 2115 2120 2125 2130 2135 2140 2145 2150 2155 2160 2165 2170 2175 2180 2185 2190 2195 2200 2205 2210 2215 2220 2225 2230 2235 2240 2245 2250 2255 2260 2265 2270 2275 2280 2285 2290 2295 2300 2305 2310 2315 2320 2325 2330 2335 2340 2345 2350 2355 2360 2365 2370 2375 2380 2385 2390 2395 2400 2405 2410 2415 2420 2425 2430 2435 2440 2445 2450 2455 2460 2465 2470 2475 2480 2485 2490 2495 2500 2505 2510 2515 2520 2525 2530 2535 2540 2545 2550 2555 2560 2565 2570 2575 2580 2585 2590 2595 2600 2605 2610 2615 2620 2625 2630 2635 2640 2645 2650 2655 2660 2665 2670 2675 2680 2685 2690 2695 2700 2705 2710 2715 2720 2725 2730 2735 2740 2745 2750 2755 2760 2765 2770 2775 2780 2785 2790 2795 2800 2805 2810 2815 2820 2825 2830 2835 2840 2845 2850 2855 2860 2865 2870 2875 2880 2885 2890 2895 2900 2905 2910 2915 2920 2925 2930 2935 2940 2945 2950 2955 2960 2965 2970 2975 2980 2985 2990 2995 3000 3005 3010 3015 3020 3025 3030 3035 3040 3045 3050 3055 3060 3065 3070 3075 3080 3085 3090 3095 3100 3105 3110 3115 3120 3125 3130 3135 3140 3145 3150 3155 3160 3165 3170 3175 3180 3185 3190 3195 3200 3205 3210 3215 3220 3225 3230 3235 3240 3245 3250 3255 3260 3265 3270 3275 3280 3285 3290 3295 3300 3305 3310 3315 3320 3325 3330 3335 3340 3345 3350 3355 3360 3365 3370 3375 3380 3385 3390 3395 3400 3405 3410 3415 3420 3425 3430 3435 3440 3445 3450 3455 3460 3465 3470 3475 3480 3485 3490 3495 3500 3505 3510 3515 3520 3525 3530 3535 3540 3545 3550 3555 3560 3565 3570 3575 3580 3585 3590 3595 3600 3605 3610 3615 3620 3625 3630 3635 3640 3645 3650 3655 3660 3665 3670 3675 3680 3685 3690 3695 3700 3705 3710 3715 3720 3725 3730 3735 3740 3745 3750 3755 3760 3765 3770 3775 3780 3785 3790 3795 3800 3805 3810 3815 3820 3825 3830 3835 3840 3845 3850 3855 3860 3865 3870 3875 3880 3885 3890 3895 3900 3905 3910 3915 3920 3925 3930 3935 3940 3945 3950 3955 3960 3965 3970 3975 3980 3985 3990 3995 4000 4005 4010 4015 4020 4025 4030 4035 4040 4045 4050 4055 4060 4065 4070 4075 4080 4085 4090 4095 4100 4105 4110 4115 4120 4125 4130 4135 4140 4145 4150 4155 4160 4165 4170 4175 4180 4185 4190 4195 4200 4205 4210 4215 4220 4225 4230 4235 4240 4245 4250 4255 4260 4265 4270 4275 4280 4285 4290 4295 4300 4305 4310 4315 4320 4325 4330 4335 4340 4345 4350 4355 4360 4365 4370 4375 4380 4385 4390 4395 4400 4405 4410 4415 4420 4425 4430 4435 4440 4445 4450 4455 4460 4465 4470 4475 4480 4485 4490 4495 4500 4505 4510 4515 4520 4525 4530 4535 4540 4545 4550 4555 4560 4565 4570 4575 4580 4585 4590 4595 4600 4605 4610 4615 4620 4625 4630 4635 4640 4645 4650 4655 4660 4665 4670 4675 4680 4685 4690 4695 4700 4705 4710 4715 4720 4725 4730 4735 4740 4745 4750 4755 4760 4765 4770 4775 4780 4785 4790 4795 4800 4805 4810 4815 4820 4825 4830 4835 4840 4845 4850 4855 4860 4865 4870 4875 4880 4885 4890 4895 4900 4905 4910 4915 4920 4925 4930 4935 4940 4945 4950 4955 4960 4965 4970 4975 4980 4985 4990 4995 5000 5005 5010 5015 5020 5025 5030 5035 5040 5045 5050 5055 5060 5065 5070 5075 5080 5085 5090 5095 5100 5105 5110 5115 5120 5125 5130 5135 5140 5145 5150 5155 5160 5165 5170 5175 5180 5185 5190 5195 5200 5205 5210 5215 5220 5225 5230 5235 5240 5245 5250 5255 5260 5265 5270 5275 5280 5285 5290 5295 5300 5305 5310 5315 5320 5325 5330 5335 5340 5345 5350 5355 5360 5365 5370 5375 5380 5385 5390 5395 5400 5405 5410 5415 5420 5425 5430 5435 5440 5445 5450 5455 5460 5465 5470 5475 5480 5485 5490 5495 5500 5505 5510 5515 5520 5525 5530 5535 5540 5545 5550 5555 5560 5565 5570 5575 5580 5585 5590 5595 5600 5605 5610 5615 5620 5625 5630 5635 5640 5645 5650 5655 5660 5665 5670 5675 5680 5685 5690 5695 5700 5705 5710 5715 5720 5725 5730 5735 5740 5745 5750 5755 5760 5765 5770 5775 5780 5785 5790 5795 5800 5805 5810 5815 5820 5825 5830 5835 5840 5845 5850 5855 5860 5865 5870 5875 5880 5885 5890 5895 5900 5905 5910 5915 5920 5925 5930 5935 5940 5945 5950 5955 5960 5965 5970 5975 5980 5985 5990 5995 6000 6005 6010 6015 6020 6025 6030 6035 6040 6045 6050 6055 6060 6065 6070 6075 6080 6085 6090 6095 6100 6105 6110 6115 6120 6125 6130 6135 6140 6145 6150 6155 6160 6165 6170 6175 6180 6185 6190 6195 6200 6205 6210 6215 6220 6225 6230 6235 6240 6245 6250 6255 6260 6265 6270 6275 6280 6285 6290 6295 6300 6305 6310 6315 6320 6325 6330 6335 6340 6345 6350 6355 6360 6365 6370 6375 6380 6385 6390 6395 6400 6405 6410 6415 6420 6425 6430 6435 6440 6445 6450 6455 6460 6465 6470 6475 6480 6485 6490 6495 6500 6505 6510 6515 6520 6525 6530 6535 6540 6545 6550 6555 6560 6565 6570 6575 6580 6585 6590 6595 6600 6605 6610 6615 6620 6625 6630 6635 6640 6645 6650 6655 6660 6665 6670 6675 6680 6685 6690 6695 6700 6705 6710 6715 6720 6725 6730 6735 6740 6745 6750 6755 6760 6765 6770 6775 6780 6785 6790 6795 6800 6805 6810 6815 6820 6825 6830 6835 6840 6845 6850 6855 6860 6865 6870 6875 6880 6885 6890 6895 6900 6905 6910 6915 6920 6925 6930 6935 6940 6945 6950 6955 6960 6965 6970 6975 6980 6985 6990 6995 7000 7005 7010 7015 7020 7025 7030 7035 7040 7045 7050 7055 7060 7065 7070 7075 7080 7085 7090 7095 7100 7105 7110 7115 7120 7125 7130 7135 7140 7145 7150 7155 7160 7165 7170 7175 7180 7185 7190 7195 7200 7205 7210 7215 7220 7225 7230 7235 7240 7245 7250 7255 7260 7265 7270 7275 7280 7285 7290 7295 7300 7305 7310 7315 7320 7325 7330 7335 7340 7345 7350 7355 7360 7365 7370 7375 7380 7385 7390 7395 7400 7405 7410 7415 7420 7425 7430 7435 7440 7445 7450 7455 7460 7465 7470 7475 7480 7485 7490 7495 7500 7505 7510 7515 7520 7525 7530 7535 7540 7545 7550 7555 7560 7565 7570 7575 7580 7585 7590 7595 7600 7605 7610 7615 7620 7625 7630 7635 7640 7645 7650 7655 7660 7665 7670 7675 7680 7685 7690 7695 7700 7705 7710 7715 7720 7725 7730 7735 7740 7745 7750 7755 7760 7765 7770 7775 7780 7785 7790 7795 7800 7805 7810 7815 7820 7825 7830 7835 7840 7845 7850 7855 7860 7865 7870 7875 7880 7885 7890 7895 7900 7905 7910 7915 7920 7925 7930 7935 7940 7945 7950 7955 7960 7965 7970 7975 7980 7985 7990 7995 8000 8005 8010 8015 8020 8025 8030 8035 8040 8045 8050 8055 8060 8065 8070 8075 8080 8085 8090 8095 8100 8105 8110 8115 8120 8125 8130 8135 8140 8145 8150 8155 8160 8165 8170 8175 8180 8185 8190 8195 8200 8205 8210 8215 8220 8225 8230 8235 8240 8245 8250 8255 8260 8265 8270

cal particle size of the emulsions was below 300 nm and the pH ranged from 3.0 to 9.5.

The examples were again ranked as described hereinabove. The organosilicon compound type, the time it took each sample to cure in minutes (min.), and the performance of each example are reported in Table II hereinbelow.

TABLE II

| Example | Organosilicon Compound Type | Cure (Min.) | Rating |
|---------|-----------------------------|-------------|--------|
| 11      | H                           | 10          | 11     |
| 12      | I                           | 10          | 12     |
| 13      | J                           | 10          | 10     |

Table II hereinabove shows that the compositions of the instant invention give excellent slickness ratings even when using a variety of catalyst types and different types of organosilicon compounds.

## Comparixon Example 1

A first emulsion was prepared in the following manner. About 2 weight percent of an aqueous solution of a mixture of two partially hydrolyzed PVA's (polyvinyl alcohols) having a degree of hydrolysis of 88% and a 4% aqueous solution viscosity of 5 centipoise (cP) and 24 centipoise (cP) at 25° C., respectively, and about 0.3 weight percent of a polyoxyethylene (10) nonyl phenol surfactant was mixed with 28 weight percent of water. Next, 13.5 weight percent of an organohydrogenpolysiloxane having the formula  $\text{Me}_3\text{SiO}(\text{MeHSiO})_5(\text{Me}_2\text{SiO})_3\text{SiMe}_3$ , and 28 weight percent of a dimethylvinylsiloxy-terminated polydimethylmethylethylvinylsiloxane having a viscosity of 350 cP were mixed and stirred. Next, the PVA-surfactant mixture was added to the siloxane mixture and stirred. This mixture was then processed through a colloid mill and diluted with 28 weight percent of water containing a biocide to form an emulsion.

A second emulsion was prepared by mixing 2 weight percent of an aqueous solution of a mixture of two partially hydrolyzed PVA's (polyvinyl alcohols) having a degree of hydrolysis of 88% and a 4% aqueous solution viscosity of 5 centipoise (cP) and 24 centipoise (cP) at 25° C., respectively, about 0.3 weight percent of a polyoxyethylene (10) nonyl phenol surfactant, and 28 weight percent of water. Next, about 40 weight percent of dimethylvinylsiloxy-terminated polydimethylmethylethylvinylsiloxane having a viscosity of 350 cP and about 1% of a platinum-containing catalyst were mixed and stirred. Next, the PVA-surfactant mixture was added to the siloxane mixture and stirred. This mixture was then processed through a colloid mill and diluted with 28 weight percent of water containing a biocide to form an emulsion.

Next, 7.5 grams of the first emulsion, 7.5 grams of the second emulsion, and 85 grams of water were mixed together and the resulting emulsion stirred.

This silicone emulsion cured in 10 minutes and the sample was ranked according to the staple pad friction procedure delineated hereinabove. The silicone emulsion attained a rating of between 4 and 5.

## Comparison Example 2

A silicone emulsion was prepared according to the disclosure of Bunge in U.S. Pat. No. 4,954,554. A first emulsion was prepared in the following manner. About 38 weight percent of a dimethylvinylsiloxy-terminated

polydimethylsiloxane having a viscosity of 450 centistokes (cst) and 2 weight percent of a mixture of an organohydrogenpolysiloxane having the formula  $\text{Me}_3\text{SiO}(\text{MeHSiO})_5(\text{Me}_2\text{SiO})_3\text{SiMe}_3$  and a dimethylsiloxane-methylhydrogensiloxane having a viscosity of 85 centistokes (cst) were mixed and stirred. About 2 weight percent of an aqueous solution of an intermediate hydrolyzed PVA having a degree of hydrolysis of 96% and a 4% aqueous solution viscosity of 30 centipoise (cP) at 25° C., a surfactant, and 29 weight percent of water were mixed and stirred. Next, the PVA-surfactant mixture was added to the siloxane mixture and stirred. This mixture was then processed through a colloid mill and diluted with 29 weight percent of water containing a biocide to form an emulsion.

A second emulsion was prepared by mixing about 2 weight percent of an aqueous solution of an intermediate hydrolyzed PVA having a degree of hydrolysis of 96% and a 4% aqueous solution viscosity of 30 centipoise (cP) at 25° C., a surfactant, and 51 weight percent of water. Next, about 40 weight percent of a dimethylvinylsiloxy-terminated polydimethylsiloxane having a viscosity of 450 cP and about 1% of a platinum-containing catalyst were mixed and stirred. Next, the PVA-surfactant mixture was added to the siloxane mixture and stirred. This mixture was then processed through a colloid mill and 7 weight percent of water containing a biocide was added to form an emulsion.

Next, 7.5 grams of the first emulsion, 7.5 grams of the second emulsion, and 85 grams of water were mixed together and the resulting emulsion stirred.

This silicone emulsion cured in 10 minutes and the sample was ranked according to the staple pad friction procedure delineated hereinabove. The silicone emulsion attained a rating of between 5 and 6. Thus the compositions of the instant invention outperformed the silicone emulsion previously described in the art.

It should be apparent from the foregoing that many other variations and modifications may be made in the compounds, compositions and methods described herein without departing substantially from the essential features and concepts of the present invention. Accordingly it should be clearly understood that the forms of the invention described herein are exemplary only and are not intended as limitations on the scope of the present invention as defined in the appended claims.

## What is claimed is:

1. A fiber treatment composition comprising:
  - (A) an allyl ester, vinyl ester, or unsaturated acetate;
  - (B) at least one organohydrogensiloxane;
  - (C) a metal catalyst; and
  - (D) an organosilicon compound having an average of at least one group per molecule selected from the group consisting of carboxy groups, ester groups, amino groups, sulfo groups, acrylate groups, epoxy groups, ether groups, and mixtures thereof.
2. A fiber treatment composition comprising:
  - (A) an allyl ester, vinyl ester, or unsaturated acetate;
  - (B) at least one organohydrogensiloxane;
  - (C) a metal catalyst;
  - (D) an organosilicon compound having an average of at least one group per molecule selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals

having from 2 to 20 carbon atoms, and mixtures thereof; and  
 (E) a dispersant selected from the group consisting of:  
 (i) surfactants; and  
 (ii) a solvent selected from the group consisting of methylene chloride, acetonitrile, toluene, xylene, white spirits, and chlorinated hydrocarbons.

3. A composition according to claim 2, wherein the composition further comprises water.

4. A composition according to claim 2, wherein (A) is selected from the group consisting of allyl acetate, linalyl acetate, and isopropenyl acetate.

5. A composition according to claim 2, wherein (B) is selected from the group consisting of bis(trimethylsilyloxy)dimethyldihydrogen disiloxane, diphenyldimethyl-disiloxane, diphenyltetakis(dimethylsiloxy)disiloxane, heptamethylhydrogen trisiloxane, hexamethyldihydrogen trisiloxane, methylhydrogen cyclosiloxanes, methyltris(dimethylhydrogensiloxy)silane, pentamethylpentahydrogen cyclopentasiloxane, pentamethylhydrogen disiloxane, phenyltris(dimethylhydrogensiloxy)silane, polymethylhydrogen siloxane, tetrakis(dimethylhydrogensiloxy)silane, tetramethyltetrahydrogenyclocleratrasiloxane, tetramethyldihydrogen disiloxane, and methylhydrogen dimethylsiloxy copolymers.

6. A composition according to claim 2, wherein (C) is selected from the group consisting of  $\text{RhCl}_3$ ,  $\text{ClRh}(\text{PPh}_3)_3$ ,  $\text{H}_2\text{PtCl}_6$ , a complex of 1,3-divinyl tetramethyl disiloxane and  $\text{H}_2\text{PtCl}_6$ , and alkyne complexes of  $\text{H}_2\text{PtCl}_6$ .

7. A composition according to claim 2, wherein (C) is a microencapsulated curing catalyst.

8. A composition according to claim 2, wherein (D) is a compound having its formula selected from the group consisting of

- (i)  $\text{R}^{13}\text{SiO}(\text{R}_2\text{SiO})_x(\text{R}^1\text{RSiO})_y\text{SiR}^{13}$
- (ii)  $\text{R}_2\text{R}^1\text{SiO}(\text{R}_2\text{SiO})_x(\text{R}^1\text{RSiO})_y\text{SiR}_2\text{R}^1$
- (iii)  $\text{RR}^1_2\text{SiO}(\text{R}_2\text{SiO})_x(\text{R}^1\text{RSiO})_y\text{SiRR}^1_2$

wherein R is a monovalent hydrocarbon or halohydrocarbon radical having from 1 to 20 carbon atoms,  $\text{R}^1$  is a group selected from the group consisting of hydroxy, hydroxylalkyl, hydroxyaryl, hydroxycycloalkyl, hydroxycycloaryl, carboxy, carboxycycloalkyl, carboxyaryl, carboxycycloalkyl, carboxycycloaryl, alkylester, arylester, cycloalkylester, cycloarylester, amino, aminoalkyl, aminoaryl, aminocycloalkyl, aminocycloaryl, acetoxy, acetoxyalkyl, acetoxyaryl, acetoxyccycloalkyl, acetoxyccycloaryl, sulfoalkyl, sulfoaryl, sulfocycloalkyl, sulfocycloaryl, alkoxy, alkoxyalkyl, alkoxyaryl, alkoxycycloalkyl, alkoxycycloaryl, acryloxy, acryloxyalkyl, acryloxyaryl, acryloxyccycloalkyl, acryloxyccycloaryl, epoxy, epoxyalkyl, epoxyaryl, epoxycycloalkyl, epoxycycloaryl, fluoro, fluoroalkyl, fluoroaryl, fluorocycloalkyl, fluorocycloaryl, alkylether, arylether, cycloalkylether, cycloarylether, olefinic hydrocarbon or halohydrocarbon radicals having from 2 to 20 carbon atoms, and mixtures thereof, x has a value of 0 to 3000, and y has a value of 1 to 100.

9. A composition according to claim 8, wherein  $\text{R}^1$  is selected from the group consisting of hydroxy, hydroxypropyl, hydroxybutyl, hydroxyphenyl, hydroxymethylphenyl, hydroxyethylphenyl, and hydroxycyclohexyl.

10. A composition according to claim 8, wherein  $\text{R}^1$  is selected from the group consisting of amino, aminopropyl, ethylene diaminopropyl, aminophenyl, ami-

noctadecyl, aminocyclohexyl, propylene diaminopropyl, dimethylamino, and diethylamino.

11. A composition according to claim 8, wherein  $\text{R}^1$  is selected from the group consisting of acetoxy, acetoxyethyl, acetoxypropyl, acetoxybutyl, acetoxyphenyl, and acetoxyccyclohexyl.

12. A composition according to claim 8, wherein  $\text{R}^1$  is selected from the group consisting of hydrogen sulfide, sulfopropyl, methylsulfopropyl, sulfophenyl, and methylsulfo.

13. A composition according to claim 8, wherein  $\text{R}^1$  is selected from the group consisting of fluoro, fluoropropyl, fluorobutyl, 3,3,3-trifluoropropyl, and 3,3,4,4,5,5,6,6,6-nonafluorohexyl.

14. A composition according to claim 8, wherein  $\text{R}^1$  is selected from the group consisting of methoxy, ethoxy, butoxy, tertiary-butoxy, propoxy, isopropoxy, methoxyphenyl, ethoxyphenyl, methoxybutyl, and methoxypropyl.

15. A composition according to claim 8, wherein  $\text{R}^1$  is selected from the group consisting of epoxide, epichlorohydrin, ethylene oxide, epoxybutane, epoxycyclohexane, epoxy ethylhexanol, epoxy propanol, and epoxy resin groups.

16. A composition according to claim 8, wherein  $\text{R}^1$  is selected from the group consisting of acryloxyethyl, acryloxyethoxy, acryloxypropyl, acryloxypropoxy, methacryloxyethyl, methacryloxyethoxy, methacryloxypropyl, and methacryloxypropoxy.

17. A composition according to claim 8, wherein  $\text{R}^1$  is selected from the group consisting of methylethylether, methylpropylether, ethylmethylether, ethylethylether, ethylpropylether, methylphenylether, ethylphenylether, isopropylphenylether, tertiary-butylpropylether, methylcyclohexylether, and ethylcyclohexylether.

18. A composition according to claim 8, wherein  $\text{R}^1$  is selected from the group consisting of carboxy, carboxymethyl, carboxyethyl, carboxypropyl, carboxybutyl, carboxyphenyl, carboxymethylphenyl, carboxyethylphenyl, and carboxycyclohexyl.

19. A composition according to claim 8, wherein  $\text{R}^1$  is selected from the group consisting of ethyl acetate, methyl acetate, n-propyl acetate, n-butyl acetate, phenyl acetate, benzyl acetate, isobutyl benzoate, ethyl benzoate, ethyl propionate, ethyl stearate, ethyl trimethylacetate, methyl laurate, and ethyl palmitate.

20. A composition according to claim 8, wherein the olefinic hydrocarbon radicals are selected from the group consisting of vinyl and hexenyl radicals.

21. A composition according to claim 2, wherein (E) is selected from the group consisting of polyoxyethylene alkyl ether, polyoxyethylene alkylphenol ether, polyoxyethylene alkyl ester, polyoxyethylene sorbitan alkyl ester, polyethylene glycol, polypropylene glycol, polyoxyalkylene glycol modified polysiloxanes, alkyltrimethylammonium hydroxide, dialkyldimethylammonium hydroxide, methylpolyoxyethylene cocoammonium chloride, and dimethyl hydroxyethylammonium methosulfate, polyethoxyethers of nonyl phenol and octyl phenol, trimethylnol ethers of polyethylene glycols, monoesters of alcohols and fatty acids, ethoxylated amines, methylene chloride, and acetonitrile.

22. A method of making a fiber treatment composition comprising:  
 (I) mixing:  
 (A) an allyl ester, vinyl ester, or unsaturated acetate,

- (B) at least one organohydrogensiloxane,
- (C) a metal catalyst, and
- (D) an organosilicon compound having an average of at least one group per molecule selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals having from 2 to 20 carbon atoms, and mixtures thereof, and
- (E) a dispersant selected from the group consisting of:
  - (i) surfactants; and
  - (ii) a solvent selected from the group consisting of methylene chloride, acetonitrile, toluene, xylene, white spirits, and chlorinated hydrocarbons.

23. A method according to claim 22, wherein the method further comprises adding water to the mixture of step (I).

24. A method of making a fiber treatment composition comprising:

- (I) mixing:
  - (i) an organosilicon compound having an average of at least one group per molecule selected from the group consisting of hydroxy groups, carboxy groups, ester groups, amino groups, acetoxy groups, sulfo groups, alkoxy groups, acrylate groups, epoxy groups, fluoro groups, ether groups, olefinic hydrocarbon or halohydrocarbon radicals having from 2 to 20 carbon atoms, and mixtures thereof, and
  - (ii) a dispersant selected from the group consisting of:

- (i) surfactants; and
- (ii) a solvent selected from the group consisting of methylene chloride, acetonitrile, toluene, xylene, white spirits, and chlorinated hydrocarbons;

(II) adding to the mixture of (I) a mixture of:
 

- (iii) an allyl ester, vinyl ester, or unsaturated acetate,
- (iv) at least one organohydrogensiloxane, and
- (v) a metal catalyst.

25. A method according to claim 24, wherein the mixture of step (II) is emulsified prior to adding the mixture of (II) to the mixture of (I).

26. A method according to claim 24, wherein the method further comprises adding water to the mixture of step (II).

27. A composition according to claim 1, wherein (A) is selected from the group consisting of allyl butyrate, allyl acetate, linallyl acetate, allyl methacrylate, vinyl acetate, allyl acrylate, vinyl butyrate, isopropenyl acetate, vinyl trifluoroacetate, 2-methyl-1-butenyl acetate, vinyl 2-ethyl hexanoate, vinyl 3,5,5-trimethylhexanoate, allyl 3-butenoate, bis-(2-methylallyl) carbonate, diallyl succinate, and ethyl diallylcarbamate.

28. A composition according to claim 2, wherein (A) is selected from the group consisting of allyl butyrate, allyl acetate, linallyl acetate, allyl methacrylate, vinyl acetate, allyl acrylate, vinyl butyrate, isopropenyl acetate, vinyl trifluoroacetate, 2-methyl-1-butenyl acetate, vinyl 2-ethyl hexanoate, vinyl 3,5,5-trimethylhexanoate, allyl 3-butenoate, bis-(2-methylallyl) carbonate, diallyl succinate, and ethyl diallylcarbamate.

\* \* \* \* \*